

Aug. 10, 1943.

R. B. DIMMICK

2,326,127

FORGED CAR WHEEL

Original Filed May 4, 1940



INVENTOR.

RALPH B. DIMMICK.

BY

*Allen & Allen*

ATTORNEYS.

## UNITED STATES PATENT OFFICE

2,326,127

## FORGED CAR WHEEL

Ralph B. Dimmick, Butler, Pa., assignor to The American Rolling Mill Company, Middletown, Ohio, a corporation of Ohio

Continuation of application Serial No. 239,691, November 9, 1938, and a division of application Serial No. 333,355, May 4, 1940. This application January 22, 1942, Serial No. 427,727

5 Claims. (Cl. 295—30)

My invention relates primarily to a process of heat treatment of ferrous wheels for railroad rolling stock and the like and an improved wheel resulting therefrom. This application is a continuation of my copending application, Serial No. 239,691, filed November 9, 1938, and is a division of my copending application, Serial No. 333,355, filed May 4, 1940. I shall describe my invention in connection with forged steel car wheels though it is not necessarily limited thereto.

The fundamental object of my invention is the provision of a process which will simultaneously bring about the following conditions in the article:

(1) The tread of the wheel has sufficient hardness to successfully withstand difficult service conditions.

(2) The hub is soft enough to permit easy machining.

(3) The tensile and fatigue strength and the ductility of the plate of the wheel are very high, adding to its factor of safety.

(4) The wheel is free of dangerously high internal stresses.

The last two of these considerations are, of course, the most important since above all the wheels must be safe. In my process the desiderata above are coincidentally achieved; and this, so far as I know, is a wholly new aspect of utility which my product possesses.

In one prior process it is the practice to heat the wheels to above the critical point and then to quench the entire wheel in a liquid, usually oil, and then uniformly to draw the temper of the entire wheel to relieve the dangerously high quenching stresses. While this process has resulted in a usable wheel, it is not all that could be desired in several respects. The chief undesirable feature is that when the wheel has been heat treated to produce a degree of hardness in the rim which will satisfactorily resist difficult service conditions, the hub is so hard as to be very difficult to machine; and the finishing of the bore becomes a very difficult and expensive operation. Such wheels also have a higher degree of stress in their plates than is desirable, probably due to the unequal cooling rate of the various parts of the wheel, resulting from their very irregular cross section.

In attempting to avoid the first of these difficulties some manufacturers have resorted to a differential quench. That is, the hot wheel is held by the hub while a quenching medium, usually water, is caused to come into contact with the rim section only. The hub and plate sec-

tions are protected from the quenching action and therefore remain soft, while the rim is hardened. While this procedure also results in a usable wheel, several new disadvantages are introduced which were not present in the uniformly quenched wheel previously described. Since only the rim section of the wheel has been quenched, the steel in the other parts of the wheel does not get the benefit of the refining action on the 5 microstructure which is afforded by a quench and a draw, and consequently the strength and ductility are inferior. Also as can readily be appreciated, this unequal quenching sets up exceptionally high stresses in the wheel. The equipment 10 for carrying out this process is, moreover, quite large and complicated and adds greatly to the inconvenience and expense of the process. Following this differential quenching operation it is customary to employ a uniform draw to relieve 15 the stresses somewhat and to improve the physical properties of the rim. The rest of the wheel 20 is little affected by this draw since it has not been quenched.

In my new process I avoid these undesirable 25 features by providing (following an over-all quench) a differential draw or tempering in which the temperature difference between the hub and the rim is carefully controlled by a differential application of heat so that the hub 30 is heated to a high enough temperature to effectively soften it while the rim is held at a sufficiently low temperature to prevent undue softening, followed by an equalization of temperatures and a slow cooling. For the best combination of 35 properties this differential draw is preceded by a uniform quench.

By following this procedure I produce a wheel 40 having a combination of maximum rim hardness to resist shelling and wear, softness in the hub to give good machining properties, and controlled stresses to provide the maximum of safety in service.

The figure is a sectional view through a type 45 of draw furnace which I may employ, showing also an exemplary heating means.

In practicing my preferred process the wheels 50 to be heat treated are first heated slowly in another furnace, not shown, to above the critical temperature, for example to around 1500° F., and are held there for a sufficient length of time for all parts of the wheel to attain a uniform temperature. This procedure of heating prior to the quench is well understood in the art and the particular heating schedule is not critical for the 55 achievement of my result.

The heated wheels are then quenched preferably in oil, although water, brine, or other fluids are effective. It is preferred that this quench be uniform over the entire wheel, that is, that no part of the wheel be protected from the rapid cooling action of the cooling medium. The principles and practice of quenching are also well understood in the art, and my invention does not contemplate the use of any particular method other than preferring a uniform quench. It is of course understood that the quench should be carried out in a manner consistent with generally understood metallurgical principles.

To accomplish the desired changes in microstructure it is only necessary to cool rapidly to below the critical temperature; but additional desirable hardness is imparted to the wheel the lower the temperature to which the wheel is quenched. This additional hardness is accompanied by increased stresses. To avoid the formation of excessively high stresses and to avoid the possibility of forming so-called shatter cracks, I prefer not to quench to below around 450° F. For reasons of commercial expediency the draw usually immediately follows the quench, and there is a saving in both heat and time if the wheel is placed into the draw furnace while still quite hot from the quench. The quench must be continued to a sufficiently low temperature, however, to give the desired hardness of the rims, and to make possible, during the draw, the temperature differential between the hubs and the rims necessary to achieve my novel result, as will now be described.

The wheels now have a microstructure refined throughout by the uniform quench. The entire wheel is hard and stressed. In my process I soften the hubs without unduly softening the rims and at the same time modify internal stresses by a differential draw which in its simplest form consists in heating the hubs hotter than the rims. In my preferred furnace, which is illustrated in the drawing, this is accomplished by the use of an internal heating means inserted within the bores of a number of stacked wheels. An exemplary arrangement for my draw furnace is illustrated in the figure. I prefer to employ a furnace which is cylindrical in form and of a diameter not much greater than the diameter of the wheels which are to be treated in it. On a suitable floor 1, I mount a cylindrical casing 2 of insulating character. The casing may, if desired, be of such character as to be removable by a crane; and the arrangement of wheels may first be made and then the casing lifted over it. Or if desired, the casing may be fixed in position and closed by means of a movable top member 3, also of insulating character. The car wheels are arranged in a vertical stack. The first wheel is placed in the furnace in a horizontal position resting on a suitable support. The second wheel is placed on top of the first, care being taken to keep the bores of the wheels in alignment. Whenever the hubs are thicker than the rims, as they usually are, I may employ spacers 5 between the rims to hold the wheels in a horizontal position. These spacers may conveniently be made of cut sections of relatively heavy 4" or 6" diameter pipe, but may also be made of other substance, metallic or non-metallic. A number of these, usually three, are placed on the top of the rim of each wheel and equally spaced around the periphery thereof, before the next wheel is placed in position.

I also commonly employ circular collars, preferably of stainless steel, placed between the plates

of the wheels, as shown at 6. The purpose of these will hereinafter be described. They may, however, be made of other substance, metallic or non-metallic. For example, asbestos composition will serve.

A third wheel is placed upon the second in the way described, and so on until the stack is completed. A furnace charge usually comprises six or seven wheels in my practice. Thermocouples 10 are inserted between the rims so that their temperature may be accurately determined during the drawing period. It is also advantageous to locate thermocouples in a position to measure the hub temperatures. Exemplary thermocouple connections are shown at 7 and 8. The cables may be thought of as connected to visual or recording instruments in a position of convenient access to the operator.

When the stack of wheels has been completed 20 in the draw furnace a heating element is positioned in the space formed by the concentric bores of the wheels. A convenient form of heating element, and one which I illustrate is an electrical resistance heater. In the figure, 9 represents the resistance element of such a heater, held by suitable heat resistive and insulating supports 10. The terminal portions of the resistance element are brought out through a top brick spacer 11, which forms a closure for a hole in the cover 3, of the furnace. If desired, a bottom brick 25 spacer 12 may be employed, the two spacers being held together by a connecting rod 13, or other suitable means which passes through the several heater supports 10.

The heating element in this form is a unitary 30 structure to be inserted and withdrawn through the hole 14 in the furnace top, and adapted to close the said hole when in position.

While an electrical heating element is most 35 convenient and most easily controlled, I am not confined to the use of such means since other types of heating devices can also be employed. A radiant tube type of heater can be used with slight modification in the furnace to provide for 40 the burner at one end and exhaust at the other. Also I find it advantageous to preheat the furnace, and sometimes to apply heat to the furnace generally, if that should appear necessary. As 45 a consequence the furnace may be provided with electrical heating elements or burners for suitable fuel and with a flue (not shown). Or the interior of the furnace may be arranged to be heated by circulation through it of hot gases derived from a burner or burners or electrical heating 50 elements located in a chamber externally of the casing 2.

In order to illustrate the method of operation 55 of my process I will describe the treatment of a lot of railway wheels of the composition specified by the Association of American Railroads, Specification M-107 which calls for carbon, .67 to .82 per cent, and manganese, 0.65 to 0.85 per cent. These wheels are first heated and uniformly quenched as above described.

In order to obtain the optimum combination 60 of rim hardness, hub softness, good physical properties in all parts of the wheel and low internal stresses made possible by my method of heat treatment I select the proper draw temperatures for the rim and hub, determining the rim draw temperature as follows:

This temperature depends on the severity of 65 the quench, the chemical composition of the steel, the desired hardness, the extent to which the quenching stresses are to be relieved, and the

time the steel is to be held at the draw temperature. For example, the more severe the quenching treatment the higher the draw temperature should be to relieve the internal stresses resulting from the quenching; the higher the carbon and manganese content the higher the draw temperature may be without appreciable loss of rim hardness; and the greater the desired relief from internal stresses the higher the draw temperature should be. In the case of a wheel of, say, 0.70 per cent carbon and 0.70 per cent manganese which has been uniformly quenched in oil and which is to have a Brinell hardness of at least 321 (a customary rim hardness for wheels of this analysis) and internal stresses not exceeding 20,000 psi, as measured in the plate of the wheel by a method to be described later, I would use a draw temperature for the rim of 800 to 900° F. and hold this for about 12 hours. However, it is possible to use a higher draw temperature for a shorter length of time, or a lower temperature for a longer time, within limits.

In order to obtain satisfactory machining properties in the hubs of such wheels I have found that it is necessary to keep the Brinell hardness thereof below 270. This can be secured by drawing the hub for at least two hours at a temperature of 1050° F. or higher. There is a practical limit to how high this temperature can go because the carbides begin to go into solution as the temperature is raised, and an undesirable coarse lamellar structure might result from the subsequent slow cooling. Preferably the draw temperature should be such that spherodization of the carbides occurs, thus leading to the optimum in machining properties. For the accomplishment of these objectives the hub should be heated to not over 1250° F. and I find that satisfactory results are obtained if it is held for three or four hours at 1100 to 1150° F.

My invention comprises supplying such means and devising the proper combination of temperatures and times as will achieve the fourfold object already recited, namely, sufficient rim hardness to resist shelling and wear, satisfactory machining properties in the hub, and good physical properties throughout the entire wheel together with low internal stresses.

Having described the selection of the draw temperatures for the rim and hub portions of the wheels, one method of carrying out the invention will now be explained according to my process and with my preferred apparatus. The heated and uniformly quenched wheels are charged into the draw furnace in the manner described, and the thermocouples placed for indication and regulation of the temperature of the hubs and rims. The electric element 9, where this type of heating means is employed, is then inserted in the bore of the wheels and the power is turned on to bring up the hub temperature as rapidly as possible to the hub draw temperature that has been selected according to the method described.

This rapid heating of the hubs is the special feature which makes possible the temperature differential between the hubs and rims when the wheels are heated as described in a heat treating mechanism such as that shown in the drawing. More specifically, my object is attained by heating the hub up to the softening temperature and holding it there long enough to obtain the desired softening, before the rim is heated high enough to be unduly softened.

This rapid heating is assisted by high wattage

or fuel input into the heating means, and by adequate enclosure of the hubs to restrict radiation from the hubs and exposed parts of the heating means between the hub faces, to the other parts of the wheels. In order to secure the difference in temperature between rims and hubs according to the preferred process already described, it is necessary of course that the wheels at the start of the drawing operation be lower in temperature than the selected drawing temperature for the rims, and the lower this initial temperature at the time the heat is first applied to the hubs, the more readily can the desired temperature difference be attained.

15 In the course of regular production, the draw furnace will naturally be heated to the selected temperature for drawing the rims of the wheels when the preceding lot of wheels is removed following the completion of the preceding cycle.

20 The furnace will cool somewhat during the charging of the next lot of wheels but it is unnecessary to cool it to room temperature before starting the drawing operation on the next lot of wheels. As I ordinarily carry out my process, 25 the wheels, after uniform quenching until they are at a temperature of about 450 to 700° F., are immediately placed in the draw furnace and the draw furnace after closing the cover will usually level off at a temperature of about 600 to 700° F.

30 Under these conditions I have found that with one form of apparatus in which I have been carrying out my process commercially, it is possible to heat the hubs to their selected softening temperature without raising the rims above their selected drawing temperature, provided that the heating means is capable of dissipating at least 16 kilowatts of electrical energy, or its equivalent if other forms of heating means are used. To provide a margin of safety I prefer to use as 35 much as 20 kilowatts or more.

These values are for average conditions with wheels of say 36" diameter and standard hubs of say 7" bore and with the use of radiation collars around the hubs as the wheels are charged 40 in the draw furnace. If the wheels are hotter when the application of heat to the hubs is started it will be necessary to apply this heat at a greater rate in order to soften the hubs without unduly softening the rims.

45 After the hubs of the wheels in the charge of six or seven wheels have been heated to at least 1050° F. and held there for at least two hours as measured by the thermocouples on the hubs of the wheels, the power is shut off on the heating element and the temperature of the hubs allowed to cool and preferably allowed to equalize with the other parts of the wheels at the selected drawing temperature for the rims. In my preferred practice the rims are never permitted to get above their proper draw temperature at any time during the drawing operation and for this purpose I employ a pyrometer controller attached to the rim thermocouple to 50 shut off the power to the hub heating element if this should be necessary.

With my preferred apparatus it is advantageous to use the equalization period and external heat is applied to heat the recirculated furnace atmosphere when necessary to maintain the selected draw temperature for the rim of the wheels. Although the time may vary with other forms of apparatus I find that, in general, it is advisable to allow at least four hours after the hub heating element is shut off for the equalization to proceed.

At the conclusion of the drawing treatment the wheels are cooled slowly in accordance with usual practice in order to avoid introduction of internal stresses by the unequal cooling rates in different portions of the wheels which would result if the wheels were cooled more rapidly. It is customary to remove the wheels from the draw furnace at the conclusion of the draw period and place them in preheated brick lined pits or tunnels where they are closely piled or stacked and require from 24 to 48 hours to cool to about 200° or 300° F.

The same result can be obtained by allowing the wheels to remain in the draw furnace and shutting off the heat while they cool to 200 or 300° F. This delays the use of the draw furnace for treating subsequent lots of wheels and is a practice followed only rarely in actual plant operation, as when the entire heat treating unit may be shut down at the end of a run.

I find that wheels of the above composition treated according to my preferred process as described, will have a rim hardness of at least 321 Brinell and a hub hardness not over 270. Furthermore, when the internal stresses are determined by the so-called dyadic-circle or rosette method as described in the Bureau of Standards Journal of Research, volume 10, 1933 R. P. 559, and volume 15, December 1935, R. P. 851, and volume 19, October 1937, R. P. 1034, the highest stress measured in the plate portion is found to be not over 20,000 psi and in most cases will be under 15,000 psi. This is a much lower stress than that obtainable by any other known methods of heat treatment which will produce hard rims and soft hubs.

Another distinguishing characteristic of wheels heat treated according to my new process is the improved microstructure in the hub portion. This consists of a partially or completely spheroidized condition of the cementite particles as contrasted with the lamellar pearlite found in wheels heat treated by other methods. Hubs of wheels that are uniformly quenched and uniformly drawn will tend to have a microstructure of finely spaced pearlite lamellae because the cooling rate is generally not great enough to produce martensite in wheels of the compositions in common use. The hubs of wheels that are non-uniformly quenched by protecting the hubs and sometimes also the plates from contact with the quenching medium, and are thereafter uniformly drawn, will have fairly coarse pearlite lamellae because of the slow cooling rate through the critical temperature range.

Thus wheels heat treated by my process are not only readily distinguishable by the spheroidized structure of the hubs but they possess the desirable properties that accompany such a structure among which are good ductility and impact resistance, high tensile and fatigue strength, and very satisfactory machinability.

My method thus produces a wheel with a rim section of sufficient strength and hardness to withstand severe service conditions, which at the same time has a hub soft enough to be readily machinable, has a desirable microstructure and physical properties, and is very low in internal stresses.

It will be understood that the showing of the heat treating apparatus is only diagrammatic and that the description which has been given of the process is only exemplary and that the invention is capable of many refinements which will readily occur to those skilled in the art. For

example, instead of inserting the heating means through the top of the draw furnace, it may be fixed to the base so that the wheels are charged by slipping the bores over the heating means. 5 The diameter of the heating means may be varied according to the size and mass of the hubs. Special precautions such as dampers in the recirculating system, if such is used, enclosures at top and bottom of the chimney formed by the 10 stack of hubs to restrict convection currents, and extra tight sealing of removable furnace covers if such are used, may be necessary in order to get the desired temperature differential between the hubs and the rims of some wheels. Although it will generally be found advantageous 15 to use the circular collars 6, in some cases the required difference in temperature between the hubs and the rims can be obtained by rough machining the faces of the hubs if they are not already smooth enough from the rough forging 20 so that they can be piled to rest hub to hub and thus prevent the radiation of heat from the heating means through any open space between the hubs and adjacent wheels, as would occur if the 25 wheels were supported by spacers placed on the rims as shown in the drawing. If the hubs are tightly enclosed, by means of circular collars or by being placed hub to hub and by closing the top and bottom of the chimney formed by the 30 stack of hubs, it is possible and may be desirable to extract heat from the rims during the hub softening part of the cycle by providing for the circulation of the furnace atmosphere around them and cooling it if necessary by the use of 35 cooling coils or other means, either in the furnace walls or externally.

Ordinarily the rims are allowed to come up to a certain temperature during the drawing operation and then are maintained at this temperature 40 during the equalization period; but for some wheels of special design it may be necessary to allow the rims to heat for a short time to a temperature above their desired draw temperature so that the hubs may be heated sufficiently to 45 soften them. Then after the hub treating means is shut off the rims are brought back to their desired draw temperature as quickly as possible by the recirculation of the furnace atmosphere. Such minor variations of my process can be made 50 without departing from the spirit of the invention, and I intend, therefore, to be limited only as indicated by the scope of the following claims.

Having now fully described my invention, what I claim as new, and desire to secure by Letters 55 Patent, is:

1. A low stress forged steel car wheel of integral character and uniform composition throughout, comprising a hub, a plate, and a rim, said wheel being characterized by a spheroidized 60 cementite structure in the hub portion thereof, and by a fine lamellar pearlite structure in the plate and rim portions thereof.

2. A forged steel car wheel of integral character and uniform composition throughout, comprising a hub, a plate, and a rim, said wheel being characterized by a Brinell hardness of at least 321 in the rim portion, a Brinell hardness not in excess of 270 in the hub portion, and in which the internal stresses in the plate portion, 65 as determined by the dyadic circle method, do not exceed 20,000 psi.

3. A low stress forged steel car wheel of integral character and uniform composition throughout, comprising a hub, a plate, and a rim, said wheel being characterized by a sphe-

roidized cementite structure in the hub portion thereof, and by a fine lamellar pearlite structure in the rim portion thereof, said wheel being further characterized by a relatively hard rim portion, a relatively soft hub portion, and a high strength plate portion.

4. A low stress forged steel car wheel of integral character and uniform composition throughout, comprising a hub, a plate, and a rim, said wheel being characterized by a spheroidized cementite structure in the hub portion thereof, and by a fine lamellar pearlite structure in the rim portion thereof, said wheel being further characterized by a relatively hard rim portion, a relatively soft hub portion, and a high strength 15

plate portion, and having a Brinell hardness of at least 321 in the rim portion, and a Brinell hardness not in excess of 270 in the hub portion.

5. A forged steel car wheel of integral character and uniform composition throughout, comprising a hub having a spheroidized cementite structure, a plate, and a rim, said wheel being characterized by a Brinell hardness of at least 321 in the rim portion, a Brinell hardness not in excess of 270 in the hub portion, and in which the internal stresses in the plate portion, as determined by the dyadic circle method, do not exceed 20,000 psi, the rim of said wheel having a fine lamellar pearlite structure.

RALPH B. DIMMICK.